

Aug. 14, 1923.

1,464,862

C. W. BALKE

METHOD AND APPARATUS RELATING TO THE PRODUCTION OF METALS

Original Filed Feb. 10, 1919



Witnesses  
Milton Lenoir  
Earl F. Pierce

Inventor  
Clarence W. Balke.  
Williams, Bradbury & Lee.  
Attorneys

## UNITED STATES PATENT OFFICE.

CLARENCE W. BALKE, OF HIGHLAND PARK, ILLINOIS, ASSIGNEE TO FANSTEEL PRODUCTS COMPANY, INC., OF NORTH CHICAGO, ILLINOIS, A CORPORATION OF NEW YORK.

## METHOD AND APPARATUS RELATING TO THE PRODUCTION OF METALS.

Application filed February 10, 1919, Serial No. 276,184. Renewed October 7, 1921. Serial No. 503,143.

To all whom it may concern:

Be it known that I, CLARENCE W. BALKE, a citizen of the United States, residing at Highland Park, in the county of Lake and State of Illinois, have invented a certain new and useful Improvement in Methods and Apparatus Relating to the Production of Metals, of which the following is a full, clear, concise, and exact description, reference being had to the accompanying drawings, forming a part of this specification.

My invention is concerned with the methods and apparatus relating to the production of metals, and is especially concerned with methods and apparatus used in the production of metals, and more specifically is concerned with the production of metals which readily oxidize at temperatures approximating their melting points.

I will describe my improved method and apparatus as used in connection with the production of misch metal, which is an alloy composed principally of cerium and certain other rare metals in combination with a small percentage of iron. This metal can be most economically manufactured by the electrolysis of cerium chloride. Prior to my invention it has been the custom to electrolyze an impure chloride of this metal in cast iron pots or crucibles. In carrying out this process a graphite or carbon electrode is used as the anode of the furnace, and has its lower end projecting into the cast iron pot or crucible. The crucible acts as the cathode of the furnace. During the operation of a furnace of this type the misch metal collects in the bottom of the crucible and the fused salt floats on top of the misch metal, thereby excluding the atmosphere from the misch metal, and thus preventing its oxidation.

After a furnace constructed in this manner has been operated for some time, it is necessary to remove the misch metal from the crucible to prevent it from contacting with the carbon or graphite electrode, and thus short-circuiting the source of electric current. By reason of the fact that the misch metal at the temperature at which it is formed in the furnace is highly inflammable, it has heretofore been the custom to remove the cast iron crucible with its content of misch metal covered by molten salt, and allow it to cool. After the misch metal has

solidified and cooled below its ignition point, it is necessary to break up the crucible in order to secure the misch metal. This method of removing the misch metal from the crucible is objectionable, first, by reason of the fact that it is expensive, as it entails the destruction of the crucible, and second, because the misch metal which is in contact with the salt is mixed with more or less of the salt.

Another objection to this method of removing the misch metal from the crucible arises from the fact that it is desirable to operate a plurality of the furnaces in which the misch metal is made, and to connect these furnaces in series with a suitable source of current. Where it is necessary to bodily remove the crucible in order to remove the misch metal formed therein, the circuit supplying the current to the plurality of furnaces must first be opened and held open until a new crucible can be substituted for the one removed, and filled with the salt and started into operation. This requires time, and during this time the remaining crucibles are cooling off more or less, and the operation of all of the furnaces is thus interfered with. It has been found desirable to keep the furnaces at a constant temperature, and this cannot be easily accomplished where it is necessary to remove the crucibles each time they are to be replaced by other crucibles.

The main objects of my invention are to provide a method and apparatus to overcome the above objections to the methods heretofore used in connection with the operation of furnaces of the type described, first, by providing a method and apparatus by means of which the misch metal can be removed from the crucibles without removing the crucibles; second, by providing means for removing the misch metal from each of a plurality of furnaces connected in series, without interrupting the flow of current through said furnaces. A further object of my invention is to provide a method and apparatus for removing the misch metal from the crucibles without exposing it to the atmosphere, and thereby eliminating losses of the metal due to oxidization thereof. A still further object of my invention is to provide means for removing the misch metal

from the crucibles, which comprises a mold for molding the misch metal into ingots of uniform size and weight.

Other objects will appear as the description progresses, reference being had to the accompanying drawings, in which—

Figure 1 is a more or less diagrammatic view showing a plurality of furnaces connected in series with a suitable electric generator, and showing my improved apparatus being used for removing the misch metal from one of the furnaces;

Figure 2 is a side elevation of one of my improved furnaces and my improved apparatus for removing the misch metal therefrom;

Figure 3 is a view similar to Figure 2, except that my improved form of furnace is shown in longitudinal section, and the vacuum pump is shown in transverse section;

Figure 4 is an enlarged detail view showing one-half of the mold removed from the other half;

Figure 5 is an enlarged sectional detail showing the means which I use to prevent molten metal being drawn into the vacuum pump; and

Figures 6 and 7 are a perspective view and a longitudinal section respectively of the end of the pipe which is used for withdrawing the molten metal from the crucible.

Similar characters of reference refer to similar parts throughout the several views.

Referring to Figure 1, wherein I have shown a plurality of furnaces comprising crucibles 10, preferably formed of cast iron, and co-acting electrodes 11, preferably formed of carbon or graphite, the reference characters 12 indicate terminal lugs formed integrally with the crucibles, which are used to make electrical connection with the cables 13 that connect the furnaces in series with each other. A shunt wound direct current generator G provides the necessary current for the furnaces. The reference character 14 indicates as a whole the means which I employ for removing the misch metal from the crucibles.

Referring to Figures 2 to 7 inclusive, this means will now be described in detail.

It will be noted from an inspection of Figures 2 and 3 that each furnace comprises a pier 15 formed of brick or other suitable material, upon which is mounted an enclosing casing 16 of sheet metal or other suitable material. This casing 16 receives the crucible 10 and is of sufficient size to leave a space between the walls of the crucible and the casing. At one side, as shown in Figure 2, the casing 16 is provided with an opening, which may be closed by a sliding gate 17 that slides in the guides 18. I provide the construction just described for the following reasons: At the temperature at

which furnaces of this type operate most efficiently to produce the misch metal, the misch metal is in a more or less plastic condition, and in order to render it sufficiently fluid to be removed by the apparatus which I am about to describe, it is necessary to raise the temperature of the misch metal to its melting point. This might be accomplished by raising the anode 11 so as to increase the resistance between the anode and the cathode, and thereby increase the energy consumed in the furnace, but I prefer to accomplish this result without any material adjustment of the anode. During the normal operation of the furnace, the filling in the space between the wall of the crucible and the casing is omitted, and the heat radiates rapidly from the crucible, thereby maintaining it at the proper temperature. When I wish to increase the temperature of the misch metal to the melting point, I fill the space between the casing and the crucible with powdered mica or powdered silocel, which is a trade name for a certain natural material having high heat insulating properties. By this means I prevent the radiation of the heat from the crucible and the temperature thereof will eventually rise to the melting point of the misch metal.

The means which I employ for removing the molten misch metal from the crucible comprises a mold 18, which I preferably form in two parts, one of which is shown in side elevation in Figure 4. These two parts are bolted together by means of bolts 19, and in order to make the mold air and liquid tight, I preferably insert a gasket (not shown) of asbestos, between the two halves of the mold. The reference character 20 indicates a source of suction, which I have conventionally illustrated in Figures 2 and 3 as being an air pump of the rotary type. This source of suction is connected with the mold by means of a rubber hose 21, and suitable pipe sections 22, 23 and 24. The reference character 25 indicates a pipe section which is adapted to be inserted in the crucible and through which the molten misch metal is removed. This pipe section is connected with the mold 18 by means of the pipe sections 26 and 27. The lower end of the pipe section 25 is slotted as shown at 26 in these figures, to provide a plurality of tongues 27, the lower ends of which rest upon the bottom of the crucible so that the misch metal can be drawn in through the slots 26. I preferably construct this pipe section of wrought iron, and if it is not allowed to remain in the molten misch metal too long, no appreciable amount of the iron will be dissolved. In some instances I have, however, made this pipe section of graphite, which is insoluble in the molten misch metal. The reference character 28 (see Figure 3) indicates a plug of misch metal, which I preferably insert in

the lower end of the pipe section 25 to prevent any of the molten salt 28 from passing into the pipe section 25 when it is being introduced into the crucible. It will of course 5 be understood that this plug will melt shortly after the insertion of the pipe 25, and thus allow the molten misch metal to pass through the pipe section 25 and into the mold.

10 I preferably connect the rubber hose 21 with the mold by means of several pipe sections, so that one of these sections, as, for instance, section 23, can be easily removed and replaced by another similar section. My 15 purpose in doing this is to provide means whereby the molten metal will be prevented from flowing into the rubber hose 21 and the vacuum pump when the mold becomes filled with molten metal. In order to accomplish this result I place a quantity of 20 copper wire or shavings 29 or other material of good heat conductivity in the pipe section 23. With this arrangement, when the mold becomes filled with molten metal and a portion 25 thereof passes into the pipe section 23, the heat is conducted away from the molten metal by means of the copper wire or shavings 29 so fast that the molten metal "freezes" and thus prevents any further 30 progress of the molten metal into the pipe 23. After a mold is filled it is removed from the pipe sections which connect it with the crucible and suction pump respectively, and another mold substituted therefor. At the 35 same time the pipe section 23 is removed and another similar section filled with copper wire or other similar material substituted therefor. It is a comparatively easy matter to punch the small plug of copper 40 mixed with misch metal from the pipe sections 23, and they can be used over again for the same purpose. I have found that it is not absolutely necessary to provide the wires or shavings for conducting the heat 45 away from the misch metal, as the pipe sections 23 will usually cool the metal sufficiently to cause it to freeze, but more metal flows into these pipes than when the wires or shavings are used, and it is more difficult 50 to displace the plug of misch metal from the pipe sections when the wires are not used.

I shall now describe briefly the operation 55 of my improved apparatus and the method of removing the misch metal from the crucibles, although this operation will probably have been understood from the above description. When sufficient misch metal has been formed in any of the crucibles, I fill 60 the space between the crucible and the casing 16 with powdered mica or silocel 30, thereby preventing radiation of heat from the crucible and raising the temperature of the misch metal to the melting point. I then 65 heat the lower end of the pipe section 25,

except at points immediately adjacent the plug 28, to a red heat, so as to prevent chilling of the misch metal by the insertion of the pipe 25. The pipe 25 is then inserted into the crucible until its lower end 70 rests on the bottom thereof, and the pump 20 is driven by any suitable means to create a suction in the mold. The atmospheric pressure upon the molten salt in the crucible and the molten misch metal thereupon 75 forces the molten misch metal through the pipe sections 25, 26 and 27 into the mold. When the mold becomes filled it is automatically prevented from passing over into the pump by the means just described, and 80 the mold is then removed and a new one substituted therefor. After sufficient metal has been removed from the crucible the operator raises the gate 17 and removes the 85 powdered mica or silocel from between the crucible and the casing, thereby permitting the crucible to cool off to the temperature at which it operates most efficiently. By means of the apparatus and method which I have just described, the molten misch metal can 90 be removed without destroying the crucible, and without in any way affecting the operation of the remaining furnaces. Furthermore, the misch metal is not exposed to atmosphere and is not oxidized. There is, 95 of course, a slight amount of air in the mold 18 which will oxidize the first portion of misch metal passing into the mold; but this amount is so small as to be entirely negligible.

100 While I have described my improved method and apparatus in connection with the production of misch metal, it is to be understood that they are capable of being used in connection with the production of 105 any metals which oxidize rapidly at temperatures approximating their melting points, and consequently my invention is not to be limited to use in connection with misch metal. Furthermore, it should be understood that the word mold as used in the specification and the claims appended hereto is not intended to be limited to a device for receiving and molding the misch metal to a definite shape, but it is intended to cover 110 any sort of a receptacle for receiving the molten metal from the crucible.

115 While I have described the details of the preferred embodiment of my invention, it is to be understood that it is capable of other 120 adaptations and modifications within the scope of the appended claims.

What I claim is:

1. The combination with a furnace for producing metals, of a casing surrounding 125 said furnace, heat insulating means, and means whereby said casing can be filled with or emptied of said heat insulating means.
2. The method of electrolytically producing an oxidizable metal such as misch metal 130

which is in a more or less plastic condition at the temperature at which it is produced, which comprises filling a plurality of furnaces with the salt from which said metal is made, passing current through said furnaces in series, raising the temperature of said furnaces beyond that at which they normally operate, by preventing the radiation of heat therefrom, and withdrawing the metal from said furnaces out of contact with the atmosphere while the electrolyzing current is passing therethrough.

3. The method of electrolytically producing a metal which is in a more or less plastic condition at the temperature at which it is produced which comprises filling a plurality of furnaces with the salt from which said metal is made, passing current through said furnaces in series, raising the temperature of said furnaces beyond that at which they normally operate, by preventing the radiation of heat therefrom, and withdrawing the metal from said furnaces, while the electrolyzing current is passing therethrough.

4. The method of electrolytically producing an oxidizable metal such as misch metal which is in a more or less plastic condition at the temperature at which it is produced, which comprises filling a plurality of furnaces with the salt from which said metal is made, passing current through said furnaces in series, raising the temperature of said furnaces beyond that at which they normally operate, and withdrawing the metal from said furnaces out of contact with the atmosphere.

5. The method of electrolytically produc-

ing a metal which comprises filling a plurality of furnaces with the salt from which said metal is made, passing current through said furnaces in series, and removing the metal from said furnaces while the current is passing therethrough.

6. The method of removing metal from an electrolytic furnace in which the metal is in a more or less plastic condition at the temperature at which the furnace normally operates, which comprises raising the temperature of said metal to the melting point by preventing the radiation of heat therefrom, and then withdrawing the molten metal from said furnace.

7. The method of removing metal from an electrolytic furnace in which the metal is in a more or less plastic condition at the temperature at which the furnace normally operates, which comprises raising the temperature of said metal to the melting point and then withdrawing the molten metal from said furnace.

8. The combination with a closed mold, of a source of suction, means for connecting said mold with said source of suction, comprising a conduit having a removable section, a second conduit for connecting said mold with a source of molten metal, and copper shavings in said removable section for preventing the flow of molten metal into said source of suction when said mold becomes filled.

In witness whereof, I hereunto subscribe my name this 15 day of January, 1919.

CLARENCE W. BALKE.

Witness:

WALTER E. CARR.